

May 31, 1966

J. H. CAIRNS

3,253,911

COPPER RICH ALLOYS

Filed Nov. 2, 1964

2 Sheets-Sheet 1

FIG. 1

ELONGATION %



Inventor  
John H. Cairns

By  
Watson, Cole, Grindle + Watson

May 31, 1966

J. H. CAIRNS

3,253,911

COPPER RICH ALLOYS

Filed Nov. 2, 1964

2 Sheets-Sheet 2

FIG. 2.

ELONGATION %



Inventor  
John H. Cairns

By  
Watson, Cole, Grindley, Watson  
Attns.

# United States Patent Office

3,253,911  
Patented May 31, 1966

1

3,253,911

## COPPER RICH ALLOYS

John H. Cairns, Stourton, near Leeds, England, assignor to Yorkshire Imperial Metals Limited, Stourton, England, a company of Great Britain

Filed Nov. 2, 1964, Ser. No. 408,169

Claims priority, application Great Britain, May 3, 1962, 16,973/62; Nov. 29, 1962, 45,143/62  
10 Claims. (Cl. 75—159)

This application is a continuation-in-part of my prior United States application Serial No. 276,375, which is now abandoned.

This invention relates to copper rich alloys such as aluminium bronze, aluminium brass, copper nickel and copper zinc, which have compositions within the copper rich alphaphase range. They may contain two or more major alloying elements and small amounts of other elements, such as iron, manganese, arsenic, to confer special properties.

Alloys of the general types described above are widely used for many applications. They have good workability at normal temperatures, although great stress is required to achieve a given amount of strain in view of their high strength. At higher temperatures the strength, and therefore the stress required to produce a given strain, are much lower but there is a "hot short range" which varies with different alloys, but in the case of copper nickel may range from about 500° to 900° C., in which there is a substantial drop in the ductility or elongation of the alloys. Because of this hot shortness it is necessary to limit the amount of working of the alloys in this range in order to avoid cracking. This is a great inconvenience and places an unfortunate restriction on the shape and size or type of component which can be produced in the alloys.

The principal object of the invention is to provide copper rich alloys of certain classes which have desirable physical properties coupled with improved working characteristics, particularly in the hot short range, and this is achieved by the addition of a small amount of zirconium to certain ranges of these alloys. Other objects will appear from a study of the following description.

It is already known to add a small amount of zirconium to certain types of alloy containing copper and/or nickel and/or aluminium, together with other elements, for various purposes, for example, to provide improved strength at high temperatures or improved hardness, or improved casting characteristics, but to the best of my knowledge it has not previously been recognised that the addition of a small amount of zirconium within a certain range produces greatly improved hot ductility in certain classes of these alloys. The improvement in hot ductility enables certain operations, such as rolling, extrusion and hot pressing and drawing, to be carried out to a much greater extent on the new alloys so that their useful range of practical application is extended.

While this improvement in hot ductility may be present to some degree, without having been recognised, in other copper-rich alloys, the classes of alloy defined below are those in which desirable physical properties are coupled with a marked improvement in hot ductility as the result of adding a small proportion of zirconium. The classification of the alloy ranges is not a recognised one and has been adopted herein only for the purpose of facilitating the definition and explanation of the invention.

The invention consists of a copper-rich alloy having high ductility in what is normally the hot short range, containing one of the following proportions of copper; about 53.5 to 63.5 percent, about 64 to 79 percent, about 85 to 95 percent; in combination with a proportion of at

2

least two of the elements nickel, iron, manganese, arsenic, zinc, aluminium; and between 0.05 and 0.5 per cent zirconium.

The invention will now be more particularly described 5 with reference to the accompanying drawings in which:

FIGURE 1 is a graph showing a comparison of the hot ductility between samples of a particular alloy with and without the presence of zirconium; and

FIGURE 2 is a graph showing a comparison of the hot 10 ductility between samples of another alloy with and without the presence of zirconium.

The classes of alloy with which the invention is concerned are as follows:

|    | Name                                               | Composition                                                                                                           |
|----|----------------------------------------------------|-----------------------------------------------------------------------------------------------------------------------|
| 15 | Class 1.—Cupro-Nickel.....                         | Nickel—10-11%.<br>Iron—0.01-2%.<br>Manganese—0.01-1%.<br>Zirconium—0.05-0.5%.<br>Copper—Remainder (about 85.5-90%).   |
| 20 | Class 2.—Cupro-Nickel.....                         | Nickel—29-33%.<br>Iron—0.01-1%.<br>Manganese—0.01-1.5%.<br>Zirconium—0.05-0.5%.<br>Copper—Remainder (about 64-71%).   |
| 25 | Class 3.—Cupro-Nickel.....                         | Nickel—35-37%.<br>Iron—1.0-2%.<br>Manganese—0.5-1.5%.<br>Zirconium—0.05-0.5%.<br>Copper—Remainder (about 59-63.5%).   |
| 30 | Class 4.—Cupro-Nickel.....                         | Nickel—40-42%.<br>Iron—0.5-2%.<br>Manganese—0.5-2%.<br>Zirconium—0.05-0.5%.<br>Copper—Remainder (about 53.5-59%).     |
| 35 | Class 5.—Copper-Zinc (70/30 Brass).                | Copper—70-73%.<br>Arsenic—0.02-0.1%.<br>Zirconium—0.05-0.5%.<br>Zinc—Remainder (about 26-30%).                        |
| 40 | Class 6.—Copper-Zinc-Aluminium: (Aluminium Brass). | Copper—76-79%.<br>Aluminium—1.8-2.5%.<br>Arsenic—0.02-0.1%.<br>Zirconium—0.05-0.5%.<br>Zinc—Remainder (about 18-22%). |
| 45 | Class 7.—Copper-Aluminium: (Aluminium Bronze).     | Aluminium—5-8%.<br>Iron—0.01-3.5%.<br>Zirconium—0.05-0.5%.<br>Copper—Remainder (about 88-95%).                        |

It is believed that the improved workability and hot ductility of the above classes of alloy is brought about by 50 the concentration of zirconium atoms at the grain boundaries of the alloys and that, in turn, this concentration results from the relatively large diameter of the zirconium atoms compared with those of copper and the other elements present in the alloys.

55 The table below shows, by way of example, the improved hot elongation obtained with alloys of the seven classes defined above by the addition of zirconium.

TABLE.—HOT ELONGATION PERCENT ON A GAUGE LENGTH OF  $4\sqrt{A}$  AREA AT TEMPERATURES OF HOT SHORTNESS

|    | Alloy                          | Alloy without Zirconium | Alloy containing Zirconium |
|----|--------------------------------|-------------------------|----------------------------|
| 65 | Class 1.—90/10 Cu-Ni.....      | 45% (850° C.).....      | 85% (850° C.).             |
|    | Class 2.—70/30 Cu-Ni.....      | 25% (950° C.).....      | 70% (950° C.).             |
|    | Class 3.—64/36 Cu-Ni.....      | 35% (1,000° C.).....    | 75% (1,000° C.).           |
|    | Class 4.—60/40 Cu-Ni.....      | 30% (1,000° C.).....    | 80% (1,000° C.).           |
|    | Class 5.—70/30 Brass.....      | 15% (400° C.).....      | 70% (400° C.).             |
|    | Class 6.—Aluminium Brass.....  | 15% (400° C.).....      | 60% (400° C.).             |
|    | Class 7.—Aluminium Bronze..... | 15% (400° C.).....      | 60% (400° C.).             |

70 As further examples of the improvement in hot ductility, FIGURE 1 illustrates by two curves the improvement ob-

tained in specific alloys of Class 2, with and without zirconium, the composition of the alloys tested being as follows:

| Element        | Alloy 1, percent | Alloy 2, percent |
|----------------|------------------|------------------|
| Nickel.....    | 31.12            | 30.85            |
| Iron.....      | 0.60             | 0.52             |
| Zirconium..... | Nil              | 0.12             |
| Manganese..... | 0.81             | 0.85             |
| Copper.....    | (1)              | (1)              |

<sup>1</sup> Remainder to 100.

FIGURE 2 shows two curves which illustrate the improvement in hot ductility provided by the addition of zirconium in a specific alloy of Class 6 above, the composition of the alloys tested being as follows:

| Element        | Alloy 1, percent | Alloy 2, percent |
|----------------|------------------|------------------|
| Copper.....    | 77.17            | 77.15            |
| Aluminium..... | 2.09             | 2.08             |
| Arsenic.....   | 0.04             | 0.04             |
| Zirconium..... | Nil              | 0.21             |
| Tin.....       | 0.01             | 0.01             |
| Lead.....      | 0.01             | 0.01             |
| Iron.....      | 0.01             | 0.01             |
| Manganese..... | 0.01             | 0.01             |
| Nickel.....    | 0.01             | 0.01             |
| Zinc.....      | (1)              | (1)              |

<sup>1</sup> Remainder to 100.

It will be noted that these last alloys contain very small amounts of tin, lead, iron, manganese and nickel. The presence or absence of these trace elements makes no appreciable difference to the properties of the alloys but they are mentioned because they were present in the alloys as tested. It will also be understood that in the specific classes of alloy mentioned earlier trace elements may also be present without appreciably affecting the particular properties.

In Classes 1 to 4 of the alloys the addition of iron and manganese confer improved resistance to corrosion in aqueous media. In Classes 5 and 6 the inclusion of a small amount of arsenic prevents corrosion by dezincification of the alloy structure. In alloys of Class 6 the addition of aluminium provides improved resistance to corrosion in many aqueous and other media. The copper aluminium alloy of this class has good resistance to oxidation and reasonable strength at elevated temperatures, this latter property being further enhanced by the addition of iron. In the Class 7 alloys larger proportions of both aluminium and iron are included for the purposes stated.

I claim:

1. A copper-rich alloy having high ductility in what is normally the hot short range, containing about 10 to 11 percent nickel, 0.01 to 2 percent iron, 0.01 to 1 percent manganese, and 0.05 to 0.5 percent zirconium, the balance being copper.

2. A copper-rich alloy having high ductility in what is normally the hot short range, containing about 29 to 33

percent nickel, 0.01 to 1 percent iron, 0.01 to 1.5 percent manganese, and 0.05 to 0.5 percent zirconium, the balance being copper.

3. A copper-rich alloy having high ductility in what is normally the hot short range, containing about 35 to 37 percent nickel, 1 to 2 percent iron, 0.5 to 1.5 percent manganese, and 0.05 to 0.5 percent zirconium, the balance being copper.

4. A copper-rich alloy having high ductility in what is normally the hot short range, containing about 40 to 42 percent nickel, 0.5 to 2 percent iron, 0.5 to 2 percent manganese, and 0.05 to 0.5 percent zirconium, the balance being copper.

5. A copper-rich alloy having high ductility in what is normally the hot short range, containing about 70 to 73 percent copper, 0.02 to 0.1 percent arsenic, and 0.05 to 0.5 percent zirconium, the balance being zinc.

6. A copper-rich alloy having high ductility in what is normally the hot short range, containing about 76 to 79 percent copper, 1.8 to 2.5 percent aluminium, 0.02 to 0.1 percent arsenic, and 0.05 to 0.5 percent zirconium, the balance being zinc.

7. A copper-rich alloy having high ductility in what is normally the hot short range, containing about 5 to 8 percent aluminium, 0.01 to 3.5 percent iron, and 0.05 to 0.5 percent zirconium, the balance being copper.

8. A copper-rich alloy having high ductility in what is normally the hot short range containing about 53.5 to 63.5 percent copper; in combination with a proportion of at least two of the metals from the group consisting of nickel, iron, manganese, arsenic, zinc and aluminium; and between 0.05 and 0.5 percent zirconium.

9. A copper-rich alloy having high ductility in what is normally the hot short range containing about 64 to 79 percent copper; in combination with a proportion of at least two of the metals from the group consisting of nickel, iron, manganese, arsenic, zinc and aluminium; and between 0.05 and 0.5 percent zirconium.

10. A copper-rich alloy having high ductility in what is normally the hot short range containing about 85 to 95 percent copper; in combination with a proportion of at least two of the metals of the group consisting of nickel, iron, manganese, arsenic, zinc and aluminium; and between 0.05 and 0.5 percent zirconium.

#### References Cited by the Examiner

##### UNITED STATES PATENTS

- 2,137,281 11/1938 Hensel et al. .... 75—159  
 2,137,282 11/1938 Hensel et al. .... 75—159  
 2,161,467 6/1939 Hensel et al. .... 75—157.5  
 2,270,716 1/1942 Morris .... 75—160  
 2,283,246 5/1942 Wise et al. .... 75—170

##### FOREIGN PATENTS

- 440,480 12/1935 Great Britain.

DAVID L. RECK, Primary Examiner.